

March 5, 1968

R. P. BARBER ET AL

3,371,983

PREWETTING CELLULOSIC FABRIC BEFORE INTRODUCTION TO DEHYDRATING  
SOLUTION OF FORMALDEHYDE REACTANT IN A CONTINUOUS PROCESS

Filed Dec. 4, 1961

2 Sheets-Sheet 1

CONTINUOUS RANGE FOR RESIN - FORMALDEHYDE FINISHING



Fig. 1

INVENTOR

RICHARD P. BARBER  
VERNON C. SMITH

BY *Cushman, Darley & Cushman*

ATTORNEYS

March 5, 1968

R. P. BARBER ETAL

3,371,983

PREWETTING CELLULOSIC FABRIC BEFORE INTRODUCTION TO DEHYDRATING  
SOLUTION OF FORMALDEHYDE REACTANT IN A CONTINUOUS PROCESS

Filed Dec. 4, 1961

2 Sheets-Sheet 2

CONTINUOUS RANGE FOR FORMALDEHYDE - RESIN FINISHING



Fig. 2

INVENTOR

RICHARD P. BARBER  
VERNON C. SMITH

BY *Cushman, Darley & Cushman*  
ATTORNEYS

1

2

3,371,983

**PREWETTING CELLULOSIC FABRIC BEFORE INTRODUCTION TO DEHYDRATING SOLUTION OF FORMALDEHYDE REACTANT IN A CONTINUOUS PROCESS**

Richard P. Barber, Mooresville, and Vernon C. Smith, Greensboro, N.C., assignors to Burlington Industries, Inc., Greensboro, N.C., a corporation of Delaware  
Continuation-in-part of application Ser. No. 136,418, Sept. 5, 1961. This application Dec. 4, 1961, Ser. No. 156,859

11 Claims. (Cl. 8—116.4)

This application is a continuation-in-part of application Ser. No. 136,418, filed Sept. 5, 1961, now abandoned.

The present invention relates to a continuous method for treating cellulosic fabrics with formaldehyde.

While formaldehyde has been employed in the past to treat cellulosic fabric, there is need for improving both the wet and dry wrinkle recovery. Furthermore, previous reactive type treatments of cellulosic fabrics, including formaldehyde treatments, degrade the fabric to an extent of over 50%.

Accordingly, it is an object of the present invention to develop an improved continuous process for treating cellulosic materials with formaldehyde.

Another object is to improve the wet wrinkle resistance of cellulosic fabrics.

A further object is to improve the dry wrinkle resistance of cellulosic fabric.

An additional object is to improve the wrinkle resistance of cellulosic fabrics while retaining 50-60% of the tensile strength.

Yet another object is to improve the wrinkle resistance of cellulosic fabrics by a reactive procedure while at the same time retaining 70% or more of the tensile strength of the fabric.

Still another object is to reduce the time of formaldehyde treatment for cellulosic fabrics.

Still further objects and the entire scope of applicability of the present invention will become apparent from the detailed description given hereinafter; it should be understood, however, that the detailed description and specific examples, while indicating preferred embodiments of the invention, are given by way of illustration only, since various changes and modifications within the spirit and scope of the invention will become apparent to those skilled in the art from this detailed description.

It has now been found that these objects can be attained by first treating the cellulosic fabric with a relatively dilute aqueous system and substantially immediately thereafter treating the cellulosic fabric with a formaldehyde solution of substantially lower water content.

By pretreating the cellulosic fabric with water there is a swelling of the fabric to make it accessible for the subsequent reaction with the formaldehyde. As a result, the reaction with formaldehyde in the next step occurs more rapidly. The amount of water retained by the fabric in this step should be between 10 and 100% by weight of the fabric. In the second step the water present in the formaldehyde solution should not be over 50% and preferably not over 20%. The solution in the second step thus acts in the nature of a dehydrating agent in that it tends to extract the impregnated water from the fabric while the formaldehyde diffuses into and reacts with the cellulosic material. The formaldehyde content of the solution is usually 5-10% but can be lower, e.g., 3%, or higher, e.g., 15%.

While the first step of the treatment is instantaneous, the second step can vary from instantaneous up to 5 minutes, the time of treatment being inversely with the

temperature in the range of room temperature to 100° C.

As the dehydrating solvent for the formaldehyde in the second step set forth above there can be employed 5 glacial acetic acid or a calcium chloride solution of from 50% concentration up to saturation, e.g., 70%, preferably 60-70%.

As a result of the two step treatment, there is obtained 10 excellent wet crease recovery together with good tensile strength retention. At the same time the time of the formaldehyde reaction is greatly reduced over that normally employed in past operations for treating the cellulosic fabric with formaldehyde.

As the cellulosic fabric there can be employed cotton, 15 linen, hemp, jute, ramie, sisal, rayons, e.g., regenerated cellulose (both viscose and cuprammonium, cellulose acetate, cellulose acetate-propionate, cellulose acetate-butylate and ethyl cellulose and mixtures of such cellulosic fabrics with each other or other fabrics, e.g., nylon, acrylic, 20 onitrile fibers or polyester fabrics. The invention is particularly applicable to the treatment of cotton fabric material such as cotton cloth.

There are two general methods for carrying out the above set forth two-step procedure.

25 In the first method the cellulosic fabric is padded to a 10-100%, preferably 60-70%, weight pick up of an aqueous solution of a strong acid, or the salt of a weak base with a strong acid, e.g., phosphoric acid, hydrochloric acid, hydrobromic acid, sulfuric acid, trichloroacetic acid, 30 formic acid, toluene sulfonic acid, ammonium chloride and ammonium sulfate. The acid strength can vary from moderate concentrations, e.g., 20% to as low as 0.01%, but preferably is between 0.5 and 6%. The preferred acid is hydrochloric acid. The acid treated fabric substantially 35 immediately thereafter is treated with the formaldehyde solution in the dehydrating solvent, e.g., glacial acetic acid or 70% calcium chloride. A small amount of acid, e.g., 0.01-2%, can be added in the dehydrating solution if desired. Also, a portion of the formaldehyde can be added 40 in the acid solution padded onto the fabric. However, a substantial portion of the formaldehyde, i.e., at least 50% should be added in the dehydrating solution. Since the initial padding with the acid solution is almost instantaneous and is usually carried out at room temperature, there 45 is no significant reaction until the fabric is placed in the dehydrating solution.

In the second method the cellulosic fabric is padded to a 50 10-100%, preferably 60-70%, weight pick up of a solution of water containing a wetting agent, preferably 0.1-1%. If the fabric is of the type which wets out, the wetting agent can be omitted and plain water employed. While anionic and cationic wetting agents can be employed, the preferred wetting agents are nonionic in character.

55 Typical examples of nonionic wetting agents are alkyl-aryl polyether alcohols such as Triton 155, p-isoctyl-phenol condensed with 10 ethylene oxide units, Arlacet C (sorbitan sesquioleate), Brij 35 (polyethylene glycol lauryl ether), Ethofats (polyethylene esters of fatty acids or rosin acids, e.g., Ethofat 3, 7, 11, 13, 15 and 19), Ethomids, e.g., Ethomid 8, 10, 12 and 14, Igepal CA (alkylphenyl polyethylene glycol ether), Myrij (polyethylene glycol stearate), Ninol 1281 (fatty acid ethanolamide), Nonionic 218 (tertiary dodecyl polyethylene glycol thioether), Pluronics (condensation products of ethylene oxide and propylene oxide having molecular weights of 400 to 4000), Span 20 (sorbitan monolaurate), Span 40 (sorbitan monopalmitate), Span 60 (sorbitan mono-stearate), Span 80 (sorbitan monooleate), Sterox CD (polyethylene glycol ester of tall oil acids), Triton X-100 (p-octylphenyl polyethylene glycol ether), Tween 20

(tris polyoxyethylene sorbitan monolaurate) and Tweens 40, 60 and 80 (the palmitates, stearates and oleates corresponding to the laurate of Tween 20).

There can also be employed anionic surface active agents such as alkyl and aryl sulfates and sulfonates, e.g., sodium alkyl benzene sulfonates having 10 to 18 carbon atoms, sodium lauryl sulfate, Aerosol OT (sodium salt of diethyl sulfosuccinate), sodium oleyl isethionate, sodium N-methyl-N-oleyl laurate, sodium salt of propylated naphthalene sulfonic acid, sodium salt of sulfonated monoglyceride of cocoanut fatty acids, Areskap 100 (sodium salt of butylphenylphenol sulfonic acid), sodium lignin sulfonate, sodium dodecyl benzene sulfonate, sodium tetradecyl sulfate and sodium dihexyl sulfosuccinate. As cationic surface active agents there can be used lauryl trimethyl ammonium chloride, cetyl pyridinium chloride and octadecyl trimethyl ammonium chloride.

After the fabric is padded with the water, with or without the wetting agent, the wet fabric substantially immediately thereafter is impregnated with a dehydrating solution, e.g., anhydrous glacial acetic acid or an aqueous calcium chloride solution of concentration from 60% to saturation, e.g., 70%. The dehydrating solution contains 5-10% of formaldehyde and also contains 0.01-20% of a strong acid, e.g., hydrochloric acid or sulfuric acid or any of the other acids previously set forth. The reaction time with formaldehyde is dependent upon the temperature in the same manner as in procedure 1.

Whether the first method or the second method is employed, it has been found that superior results are obtained by applying 2-18% of a crease-proofing resin. The crease-proofing resin can be applied before or after the formaldehyde treatment but is preferably applied first. The addition of the resin not only increases the dry wrinkle recovery angle but also increases the wet crease angle. Thus, reaction of formaldehyde aided the resin in increasing the dry wrinkle recovery angle while the resin correspondingly aided the formaldehyde in increasing the wet angle recovery. By using the resin treatment followed by the two step procedure of formaldehyde application of the present invention the decrease in tensile strength of the fabric can be limited to 30%. This is a much lower decrease in tensile strength than any of the previously employed formaldehyde or other reactive type treatments of cellulosic fabric for improving wrinkle resistance.

As the resin there can be employed any of the curable crease-proofing resins. These include the urea-aldehyde, e.g., urea-formaldehyde resin, dimethylolurea, dimethyl ether of urea-formaldehyde resin, aminotriazine-aldehyde resins, e.g., melamine-formaldehyde resins including alkylated melamine-formaldehyde, trimethylol melamine, methylated trimethylol melamine, tetrahydro-5-hydroxy-2-(1H)-pyrimidone-formaldehyde resin, cyclic ethylene urea-formaldehyde, e.g., dimethylol ethylene urea, uron-formaldehyde resins, e.g., dimethylol uron, Aerotex 23 (a triazine-formaldehyde resin believed to be a melamine-formaldehyde type resin), Rohm and Haas Resin N-17 (a triazone-formaldehyde resin, e.g., dimethylol ethyl triazone), Dextraset 48 (a uron-formaldehyde resin), Eponite 100 (believed to be a butadiene diepoxide). Other polyepoxides can be used including bisphenol-A epichlorhydrin, 1,4-bis (2,3-epoxypropoxy) benzene, 1,3-bis (2,3-epoxypropoxy) octane, ethylene glycol diglycidyl ether, as well as any of the other polyepoxides set forth

in Schroeder et al. Patent 2,774,691. Other crease-proofing agents such as those set forth in "Textile Industries," October 1959, pp. 116-127, can also be used.

The time and temperature for curing the resins are those conveniently employed in the art. For convenience, cures at 350° F. (178° C.) for 1½ minutes were employed in the specific examples.

Unless otherwise indicated, all parts and percentages are by weight.

10 In the drawings:

FIGURE 1 is a schematic diagram of a preferred continuous operation according to the invention; and

FIGURE 2 is a schematic diagram of an alternative continuous operation.

15 Referring to FIGURE 1, the cotton cloth was passed substantially instantaneously through the resin padding tank 1 containing, for example, an aqueous solution of melamine-formaldehyde. The cloth picked up 4% of resin. It then went to drier 2 where it remained for 1½ minutes 20 at 300° F. (149° C.) and then to the curing oven 3 where it remained for 1½ minutes at 350° F. (178° C.). The cotton cloth containing the cured resin next went substantially instantaneously through formaldehyde catalyst padding solution 4 which was 1.5% aqueous hydrochloric acid at room temperature. The cloth picked up approximately 60-70% of its own weight of the acid solution and then passed into formaldehyde reactor 5 maintained at 50° C. The reactor contained 70% calcium chloride, 5% formaldehyde and 25% water. It took 30 seconds for the 25 cloth to run through the reactor. The fabric was then treated in conventional fashion by passing through 10% aqueous ammonia for 30 seconds in neutralization chamber 6 and then washed in water for 30 seconds in washing operation 7. The cloth was then dried in drier 8 for 30 several minutes at 110° C. to remove the water.

35 Referring to FIGURE 2, the cotton cloth was passed substantially instantaneously through the formaldehyde catalyst padding solution 9 containing 2% aqueous hydrochloric acid at room temperature. The cloth picked up 60-70% of its own weight of the acid solution and then passed into formaldehyde reactor 10 maintained at 50° C. The reactor contained 8% formaldehyde dissolved in anhydrous glacial acetic acid. It took about one minute for the 40 cloth to run through the reactor. The fabric then passed through 10% aqueous ammonia for 30 seconds in neutralization chamber 11 and then was washed with water for 30 seconds in washing operation 12 and dried for several minutes at 110° C. in drier 13. The dried formaldehyde treated fabric then passed substantially instantaneously through resin padding tank 14 containing, for example, an aqueous solution of methylated urea-formaldehyde. The cloth picked up 6% of resin. It then went to drier 15 where it remained for 1½ minutes at 300° F. (149° C.) and then to the curing oven 16 where it remained for 1½ minutes at 350° F. (178° C.). The 45 cotton cloth was then washed in washing operation 17 to remove any remaining acid and again dried.

50 Table 1 shows the results obtained by treating cotton cloth with an aqueous solution of hydrochloric acid to a pick up of 60-70% of the weight of the fabric followed by reaction with a glacial acetic acid solution containing 8% formaldehyde. No resin treatment was utilized. Examples 2-6 in the table are in accordance with the invention and Examples 1 and 7 are controls. Example 7 55 shows the properties of the cloth without any treatment.

TABLE I

| Example | Temperature (° C.) | Time (min.) | Pad Solution (60-70% Pickup) | Tensile Strength, W & F (lbs.) | Wet Wrinkle Recovery, W & F (Monsanto) |
|---------|--------------------|-------------|------------------------------|--------------------------------|----------------------------------------|
| 1-----  | 90                 | 5           | 100% water-----              | 63 X 51                        | 2.88 X 2.82                            |
| 2-----  | 90                 | 1           | 0.5% HCl-----                | 37 X 25                        | 3.65 X 3.62                            |
| 3-----  | 70                 | 1           | 1.0% HCl-----                | 37 X 25                        | 3.58 X 3.5                             |
| 4-----  | 70                 | 1           | 0.5% HCl-----                | 43 X 34                        | 3.48 X 3.45                            |
| 5-----  | 50                 | 1           | 1.5% HCl-----                | 60 X 39                        | 3.3 X 3.3                              |
| 6-----  | 30                 | 1           | 6.0% HCl-----                | 44 X 35                        | 3.44 X 3.4                             |
| 7-----  |                    |             |                              | 61 X 51                        | 3.05 X 2.90                            |

Table 2 shows the results obtained by treating cotton cloth with a 1% aqueous solution of Triton 155 (higher alkyl aryl monoether of polyethylene glycol) to a pick up of 60-70% of the weight of the fabric followed by reaction with a glacial acetic acid solution containing 8% formaldehyde and the indicated amounts of HCl. Examples 8-18 are in accordance with the invention. Example 19 is a comparison example wherein the cotton cloth was in the dry state before entering the formaldehyde reactor (i.e., there was no previous water pick up) and Example 20 shows the properties of the cloth without any treatment.

product had a tensile strength (lbs.) 47 x 37 (W & F), dry wrinkle recovery (W & F) of 2.7 x 3.0 and a wet wrinkle recovery (W & F) of 3.52 x 3.52.

*Example 31*

5 Cotton cloth was padded with 1% aqueous HCl to a 60-70% pick up and was immediately thereafter impregnated with a solution containing 70% calcium chloride, 10% formaldehyde and 20% water at 60° C. for 1/2 minute.

*Example 32*

Cotton cloth was padded in a substantially instantane-

TABLE 2

| Example | Temperature (° C.) | Time (min.) | Percent HCl | Tensile Strength Filling (lbs.) | Wet Wrinkle Recovery, W & F (Monsanto) |
|---------|--------------------|-------------|-------------|---------------------------------|----------------------------------------|
| 8       | 90                 | 1/2         | 0.5         | 18                              | 3.72 x 3.67                            |
| 9       | 90                 | 1           | 0.5         | 15                              | 3.93 x 3.93                            |
| 10      | 70                 | 1           | 0.5         | 24                              | 3.73 x 3.76                            |
| 11      | 50                 | 1           | 0.5         | 31                              | 3.4 x 3.52                             |
| 12      | 30                 | 1           | 0.5         | 39                              | 3.2 x 3.2                              |
| 13      | 90                 | 3           | 0.01        | 34                              | 3.5 x 3.4                              |
| 14      | 70                 | 3           | 0.05        | 31                              | 3.5 x 3.4                              |
| 15      | 50                 | 3           | 0.2         | 27                              | 3.5 x 3.5                              |
| 16      | 70                 | 1/2         | 0.4         | 27                              | 3.5 x 3.5                              |
| 17      | 70                 | 1/2         | 2.0         | 28                              | 3.76 x 3.74                            |
| 18      | 30                 | 5           | 2.0         | 33                              | 3.63 x 3.65                            |
| 19      | 30                 | 5           | 2.0         | 32                              | 2.82 x 3.09                            |
| 20      |                    |             |             | 51                              | 3.06 x 2.90                            |

Table 3 shows the results obtained by padding cotton cloth with 6.0% aqueous hydrochloric acid to a pick up of 60-70% by weight of the cloth followed by impregnation with 8% formaldehyde in glacial acetic acid for 1-3 minutes at 30-35° C. followed by neutralization, washing and drying and then padding with an aqueous solution of Aerotex 23 resin to a pick up of 10% by weight of the cloth in Examples 21-24 and to a pick up of 8% in Examples 26-29. Example 25 was a comparison example wherein the fabric was treated only with 10% of the resin (no formaldehyde treatment). In Examples 21-29 after the resin padding operation, the cloth was dried for 1 1/2 minutes at 300° F. (149° C.) and then cured for 1 1/2 minutes at 350° F. (178° C.).

TABLE 3

| Example | Tensile Strength, W & F (lbs.) | Dry Wrinkle Recovery, W & F (Monsanto) | Wet Wrinkle Recovery, W & F (Monsanto) |
|---------|--------------------------------|----------------------------------------|----------------------------------------|
| 21      | 39 x 23                        | 3.67 x 3.71                            | 3.59 x 3.51                            |
| 22      | 45 x 28                        | 3.59 x 3.6                             | 3.6 x 3.5                              |
| 23      | 45 x 25                        | 3.55 x 3.55                            | 3.6 x 3.53                             |
| 24      | 45 x 23                        | 3.64 x 3.64                            | 3.67 x 3.65                            |
| 25      | 50 x 34                        | 3.29 x 3.32                            | 3.38 x 3.38                            |
| 26      | 46 x 29                        | 3.59 x 3.59                            | 3.5 x 3.5                              |
| 27      | 42 x 30                        | 3.45 x 3.55                            | 3.59 x 3.52                            |
| 28      | 41 x 25                        | 3.53 x 3.52                            | 3.63 x 3.58                            |
| 29      | 40 x 27                        | 3.61 x 3.6                             | 3.58 x 3.61                            |

35 ous manner with 1.3% of aqueous HCl at room temperature to a pick up of 60-70% by weight of the fabric. The cloth then passed through a solution containing 60% calcium chloride, 5% formaldehyde, 1% HCl and 34% water for 45 seconds at 50° C. The product had the following properties:

40 Tensil strength (filler) \_\_\_\_\_ lbs. 33  
Dry wrinkle recovery (W & F) \_\_\_\_\_ 3.1 x 2.8  
Wet wrinkle recovery (W & F) \_\_\_\_\_ 3.4 x 3.5  
Formaldehyde pick up \_\_\_\_\_ percent 0.354

45 50 Table 4 shows the results obtained using the procedure illustrated in FIGURE 1 with four different commercially available crease-proofing resins. The resins were padded onto the cotton cloth in an amount of 8%, the cloth dried for 1 1/2 minutes at 300° F. (149° C.) and then cured at 350° F. (178° C.) for 1 1/2 minutes. The cloth was then padded with 1.5% aqueous HCl followed immediately by impregnation with a mixture of 70% calcium chloride, 5% formaldehyde, 0.2% HCl and the balance water at 55 50° C. for 1 minute.

TABLE 4

| Example | Resin         | Tensile Strength (Filling) lbs. | Dry Wrinkle Recovery, W & F | Wet Wrinkle Recovery, W & F |
|---------|---------------|---------------------------------|-----------------------------|-----------------------------|
| 33      | Aerotex 23    | 32                              | 3.1 x 3.08                  | 3.67 x 3.58                 |
| 34      | Rhonite N-17  | 34                              | 3.0 x 3.0                   | 3.38 x 3.48                 |
| 35      | Dextrastex 48 | 35                              | 3.18 x 3.09                 | 3.45 x 3.48                 |
| 36      | Eponite 100   | 37                              | 2.82 x 2.85                 | 3.38 x 3.32                 |

*Example 30*

Using the procedure shown in FIGURE 1, there was padded onto cotton cloth 4% of Aerotex 23. The resin was cured for 1 1/2 minutes at 350° F. (178° C.). There was then padded on the cloth a 1% aqueous HCl solution to a pick up of 60-70% by weight of the cloth followed by impregnation with 8% formaldehyde in glacial acetic acid for 2 minutes at 50° C. There was a pick up of 0.670% formaldehyde on the fabric. The

70 75 In the present specification and claims when the percent of calcium chloride is referred to it is calculated as calcium chloride hexahydrate which is the commercially available form.

We claim:

1. A continuous process for increasing the wet wrinkle recovery of a cellulosic fabric comprising treating the fabric with an aqueous medium in which water is the sole essential liquid until the fabric contains 10-100% of its own weight of added water, substantially immediately

thereafter passing the wet fabric into a dehydrating solution of formaldehyde at a temperature up to 90° C. for a period of up to 5 minutes whereby the formaldehyde reacts with said fabric to improve the wet wrinkle recovery, washing the thus treated fabric with water and then drying said fabric.

2. A process according to claim 1 in which the fabric is a cotton fabric.

3. A process according to claim 1 wherein the dehydrating solution is one selected from the group consisting of (a) an aqueous solution containing at least 50% calcium chloride, calculated as calcium chloride hexahydrate, and at least 3% formaldehyde; and (b) anhydrous acetic acid containing at least 3% formaldehyde.

4. A process according to claim 3 wherein the treatment with formaldehyde is carried out in the presence of an acid catalyst and the fabric, directly after the formaldehyde treatment, is passed through an acid-neutralizing bath and then washed and dried.

5. A process according to claim 4 wherein the acid catalyst is present in the aqueous medium and said medium includes not more than 50% of the formaldehyde requirements for said process.

6. A process according to claim 4 wherein the acid catalyst is in the dehydrating solution and the aqueous medium includes a fabric wetting agent.

7. A process according to claim 4 including the application of a crease-proofing resin to said fabric prior to the formaldehyde treatment.

8. A process according to claim 4 including the application of a crease-proofing resin to said fabric after the formaldehyde treatment.

9. The process of claim 4 wherein said acid catalyst is hydrochloric acid, and the dehydrating solution is an aqueous solution of calcium chloride at a temperature of 50°-90° C.

10. The process of claim 9 wherein the treatment with said dehydrating solution takes from 30 seconds to 1 minute.

11. The process of claim 10 wherein the cloth is kept in open width throughout.

#### References Cited

##### UNITED STATES PATENTS

|           |        |                 |       |           |
|-----------|--------|-----------------|-------|-----------|
| 2,080,043 | 5/1937 | Heckert         | ----- | 8-116.3   |
| 995,852   | 6/1911 | Eschalier       | ----- | 8-116.4   |
| 2,338,983 | 1/1944 | Thackston       | ----- | 8-116.3   |
| 2,593,207 | 4/1952 | Silver          | ----- | 8-116.3   |
| 3,046,079 | 7/1962 | Reeves          | ----- | 8-116.4   |
| 2,689,194 | 9/1954 | Russell         | ----- | 8-116.4 X |
| 2,922,768 | 1/1960 | Mino et al.     | ----- |           |
| 2,243,765 | 5/1941 | Morton          | ----- | 8-116.4   |
| 3,189,404 | 6/1965 | Takizaki et al. | ----- | 8-116.4   |
| 3,175,875 | 5/1965 | Gagarine        | ----- | 8-116.4 X |
| 3,265,463 | 8/1966 | Barber et al.   | ----- | 8-116.4 X |
| 3,038,777 | 6/1962 | Daul et al.     | ----- | 8-116.4   |

##### FOREIGN PATENTS

|         |        |                |
|---------|--------|----------------|
| 462,005 | 3/1937 | Great Britain. |
| 568,258 | 3/1945 | Great Britain. |

##### OTHER REFERENCES

- Reeves et al., American Dyestuff Reporter, vol. 49, No. 25 18, 27-32 Sept. 5, 1960.  
 Chance et al., Textile Research Journal, vol. 31, 366-376 April, 1961.  
 Goldthwait, Textile Research Journal, vol. 21, 55-61 January 1951.  
 30 Datye et al., Textile Research Journal, vol. 30, 72-73 January 1960.  
 Reeves et al., Textile Research Journal vol. 30, 179-192 March 1960.  
 35 Daul et al., Textile Research Journal, vol. 23, 738-747 August 1954.  
 J. TRAVIS BROWN, *Acting Primary Examiner.*  
 A. LOUIS MONACELL, J. S. LEVITT, J. T. BROWN,  
 Examiners.  
 40 J. CANNON, *Assistant Examiner.*